

July 16, 1946.

W. LUDEL

2,404,184

WHEEL DRESSING TOOL AND METHOD FOR MAKING THE SAME

Filed June 28, 1944



INVENTOR

William Ludel

BY

J. Barnes

ATTORNEY

44-120

Patented July 16, 1946

2,404,184

# UNITED STATES PATENT OFFICE

2,404,184

## WHEEL DRESSING TOOL AND METHOD FOR MAKING THE SAME

William Ludel, New York, N. Y.

Application June 28, 1944, Serial No. 542,525

3 Claims. (Cl. 125—39)

1

This invention relates to an abrasive wheel dressing tool, more particularly to an abrasive wheel dressing tool employing diamonds as the wheel dressing abrading material and to a method for preparing the same.

Known to me is the provision of tools employing diamonds for dressing grinding wheels where these are made of Carborundum or like material in which the abrasive particles of this constitution are united by some bond or binder and are formed or cast into wheels. When these wheels become scored or otherwise irregularly worn, they are "dressed" by a dressing tool, as known in the art, in which a tool carrying a harder material than the abrasive of the wheel is employed to refinish the surface.

There has been devised, as known to me, dressing tools comprising a rod-like member formed at one end with a cup or socket within which diamond dust or diamond fragments are held by a matrix of alloy. The cup or socket is filled either by pouring the mixture of molten metal and the diamond dust into the cup or socket, or by molding a mixture of the diamond dust and pulverized alloying material to form, under sintering temperatures, a bond for the diamond dust particles, thereby providing a formed abrasive material by the combined action of heat and pressure. These dressing tools have not met with success due to an inefficient use of the diamond dust or particles. Use of these tools has resulted in glazing of the dressing tool surface, tending to favor the use of a single large diamond for the dressing operation and more frequently employing a cluster of a small number of diamonds in some mechanical holder to effect the wheel dressing operation.

The prior procedure known to me involving a pouring of a mixture of alloying material and diamond dust or particles or the molding process is not efficient because of the haphazard arrangement of the diamond dust, the failure to take into account the weakness of diamond fragments and the reliance merely upon the characteristic hardness of the diamond dust or fragments in relation to the abrasive of the wheel to be dressed.

I have discovered that within limited and rather critical sizes of diamond crystals of octahedron shape and alloying material, which will hereafter be described more particularly, and which may be heated to secure a free-flowing, extremely liquid material, that a more efficient wheel dressing tool may be made than heretofore. I have discovered that diamonds of octahedron shape in an alloy at the liquid stage adjust them-

2

selves in a more efficient abrading position, especially under heat treatment tending to effect ebullition of the alloy.

Still more particularly I have discovered that with diamonds of a size within specified ranges and of octahedron shape, an ebullition of the matrix alloy free from exterior influences tending to otherwise stir up the liquid mass, causes the particles of diamond of octahedron shape to adjust themselves, prior to setting of the alloying matrix, to produce a highly efficient wheel dressing tool.

Accordingly, it is an object of my invention to provide a wheel dressing tool employing diamond crystals held in a wheel tool by a metallic matrix to dispose the crystals of diamonds to provide a highly efficient wheel dressing surface or mass.

Still further it is an object of my invention to provide a method for forming a wheel dressing tool in which diamond crystals are embedded in a metallic matrix under conditions which will permit the diamond crystals to arrange themselves freely and assume positions within the matrix most effective for wheel dressing operations, unaltered by the means to heat the matrix metal, and uninhibited to move to have the crystals assume the most effective cutting position by contact with adjacent crystals.

Thus, it is an object of my invention to provide a tool holder with a cup or socket for exposing a wheel dressing surface or end, in which diamond crystals are held within a matrix of metallic alloy in which the particles assume the most effective cutting position by freedom of movement within the matrix alloy by melting the alloy, before cooling, to an extremely liquid condition.

Still further objects of my invention reside in the provision of a wheel dressing tool which is highly efficient in its wheel dressing action.

To obtain these objects and such further objects as may appear herein or may be hereinafter pointed out, I make reference to the accompanying drawing forming a part hereof in which:

45 Figure 1 is a side elevation partly in section diagrammatically illustrating the apparatus for forming my wheel dressing tool;

Figure 2 is a magnified fragmentary section of the working end thereof;

50 Figure 3 is a plan view of the working end of my wheel dressing tool; and

Figure 4 is an end elevation showing the tool applied for grinding wheel dressing operations.

In accordance with my invention, by reference 55 to the drawing, I provide a tool holder body 10

which is preferably a rod of cold rolled steel of sufficient length to serve for manual holding or tool rest mounting, one end of which is restricted at 11 and formed with a socket or cup 12, defined by a chamfered portion 13 at its periphery. The restricted portion 11 is then disposed within the high frequency induction heating elements 14 and 15, the terminals of which, 16 and 17, are formed with conductors 18 and 19 to a suitable source of electricity to provide high frequency current suitable for inducing sufficient heat to convert the matrix alloy to extreme fluidity within the socket 12 of the tool holder body 10. In this position I then insert a strip or filament of alloying material 20, which, at the temperature of the induction heating apparatus, serves to melt a small portion thereof to provide a layer 21 of molten alloying metal. Thereupon the strip of metal 20 is removed and there is added to the socket 12 a few crystals of diamond particles 22.

Thereupon the strip of alloying material 20 is reinserted within the socket 12 to provide another layer of molten material. Another layer of diamond crystals 23 are then sprinkled within the socket. This procedure is continued to supply alternating layers of the alloying metal in molten form followed by a sprinkled layer 24 of diamond crystals until the socket 12 has been filled, such as by providing another or superimposed layer of diamond crystals 25.

Thereupon the induction heating element is brought into play to bring the alloying metal to extreme fluidity to the point where there is evidence of ebullition. During this operation the diamond crystals are free to move and in instances show evidence of rising and falling within the liquefied alloy. During this action the particles adjust themselves to position the effective cutting edges 26 in the direction of the rim 13.

A rather sparse supply of diamond crystals, to the point where there is sufficient space for free and independent adjustment of the crystals in relation to the liquefied alloy matrix, is one of the desirable phases of my procedure whereby the crystals may adjust themselves and assume the most desirable position for the wheel dressing operation.

In the practice of my invention, I have discovered that diamonds in the crystallizing form and of substantially true octahedron shape, provide the most desirable result and these crystals are carefully selected from diamonds as mined to be free from fracture or chips and are therefore distinguishable from diamond dust or chippings, flakes, or the like, which are by-products of the diamond industry in connection with brillianting or polishing diamonds for their ornamental and optical properties. In connection with a tool holder which exposes a working surface adjacent the periphery 13 of approximately three eighths of an inch in diameter, I have found that in relation to the particular alloy which I will describe hereafter, that selected diamond crystals of octahedron shape and of the size approximately 25 to 35 to the carat, preferably 30 per carat, best serve my purposes. Chips and flakes are to be avoided. Sizes of crystals much above 25 to the carat or much below 35 to the carat do not respond favorably with the alloy I will now describe.

The alloy which I have found as having a specific relationship to the diamond crystals of the size as described, is an alloy made under the patent to Leach, Patent No. 1,829,903, assigned to

Handy & Harmon, and is known on the market under the trade-mark "Sil-Fos."

This is an alloy which consists of silver, varying from 10% to 25%, copper from 67% to 88%, and phosphorus varying from 2% to about 8%. The alloy starts to melt at about 1,185° F. (641° C.) and is extremely liquid and free-flowing at 1,300° F. (704° C.) to 1,340° F. (727° C.).

At temperatures somewhat higher than 1,340° F. (727° C.) there is evidence of ebullition, which is to be noted in connection with my process in one of its phases. The characteristic features of the alloy described in relation to the diamond crystals resides in the extreme fluidity and free-flowing character of the alloy at the temperatures induced by the induction heater and the evidence at higher temperatures of ebullition. Extraneous disturbing influences are avoided by the induction heating method which I have described, which, by reason of the method of adding the diamond crystals in their relatively sparse condition and the fluidity of the alloy, serves to permit the particles to assume a position during heating to dispose and position the sharper points 26 in the direction of the working edge 13 as the tool holder body 10 is held vertically during the heating operation. The pyramidal side walls of the diamond crystals are likewise effective as the diamonds wear down in the wheel dressing operation as shown in Figure 4 where the tool 10 is pressed against the periphery of the grinding wheel W.

Upon cooling of the tool and its contents, the alloy matrix retains the diamond crystals in the most effective position described. This effect is sharply in contrast with methods heretofore known to me, involving either the pouring of a molten alloy and diamond particles to within the tool holder cavity, a molding mixture of the diamond alloy and sintering of the matrix alloy, or a setting of the diamonds in a matrix binder alloy. Freedom of movement of the particles in the matrix alloy in the fluid condition contributes to the adjustment of the particles to achieve the most desirable and effective direction and is not to be confused with a heating of a matrix alloy which merely fills and flows into the interstices of a socket filled with diamond dust or particles.

By the use of the induction heater which I have described and preferably employ, alteration by oxidation of the alloying material, is substantially avoided. The formation of an oxidized coating is likewise not experienced which, in accordance with prior methods, I believe, inhibits the free movement of the particles to their most effective abrading position.

While, from my experience, the Sil-Fos alloy has been found to give the most satisfactory results, it is clear that other alloys may suggest themselves to those skilled in the art from some of the comparable properties during the heating operation which I have described by reference to Sil-Fos. However, I have found that the silver-copper-phosphorus alloy which I employ additionally responds desirably during the wheel dressing operation, in that there is a kind of softness in the matrix formed by this alloy which results in doing clean work without gathering detritus as a result of the wheel dressing operation, and therefore, with the matrix alloy which I employ, the effectiveness of the wheel dressing operation is not limited, but does clean cutting of the wheel to be dressed to the last layer of the diamond crystals in the socket 12 as the side walls 11 are worn down in the finishing operation.

I maintain the induction heater in operation during the building up of the batch within the socket 12 and my method of maintaining a liquid condition of the matrix alloy as each layer of diamond crystals is added avoids any tendency to fracture the diamond, such as is known to result by successive heating and cooling of the matrix alloy to embed diamond dust or crystals in wheel dressing tools by a procedure amounting to setting of the diamonds in the alloy and involving building up layers of alloying material, then setting diamond dust therein by removing the source of heat, followed by alternate steps of adding an additional layer of alloy and diamond dust. Each step of removing the heat by this process known to me has a deleterious effect on the diamonds due to shrinkage and expansion of the heated alloy.

The number of diamonds employed within the socket is dependent upon the size of the wheel dressing tool and the particles are limited substantially to provide the degree of sparseness and spacing of the crystals in relation to each other whereby free movement is permitted to effect the adjustment of the crystals within the fluid alloy matrix during heating operation.

The diamond crystals to be employed are those which are free from extraneous minerals on the surfaces thereof. Mechanical cleaning may be resorted to, though frequently dipping in acids to remove extraneous matter is found to be practiced by the suppliers and is found to be desirable. While this special treatment is practiced, it is to be understood that cleanliness to insure direct contact of the alloy with the diamond crystal is the object to be attained by the cleaning process.

By my method, whereby diamond crystals or grains of octahedron shape within the range of sizes between 25 to 35 to the carat, preferably 30 to the carat, an unpredictable relationship to the preferred alloy, which I have described, exists, in that the crystals assume a desirable position in relation to the working surface and are not subject to any differential and detrimental shrinkage force in cooling of the alloy until the final mass has been formed and the finishing tool is free from any evidence of inadequate surface contact between the matrix and the diamond crystals.

Furthermore, by the use of the alloy constituent for the matrix as herein described, a fast grinding wheel finishing operation is exhibited by my finishing tool, free from any tendency to gather detritus limiting the cleaning-up action of the dressing tool in its action upon the grinding wheel.

While I do not wish to be restricted to the following explanation, the procedure described shows evidence of orientation of the most effec-

tive cutting points of the octahedron crystals in the direction of the working surface by a flotation of the crystals in the matrix during the heating operation by the induction heater and this orientation is aided to some extent by the ebullition during the final heating steps of the filled socket after the successive layers of molten alloy and crystals have been built up to fill the socket.

Accordingly, I have provided a wheel dressing tool comprising a plurality of diamond crystals oriented with their most effective cutting edges in the direction of a working surface of the wheel dressing tool and held therein in an alloying matrix. Other advantages will readily appear to those skilled in the art.

Having thus described my invention and illustrated its use, what I claim as new and desire to secure by Letters Patent is:

1. The method of making a wheel dressing tool in which a plurality of diamond crystals are bonded by an alloy matrix within a form, the steps which include providing said form with a charge of diamond crystals and an alloy consisting of silver varying from about 10% to 25%, copper varying from about 67% to about 88%, and phosphorus varying from about 2% to about 8%, the diamonds being sparsely distributed, and heating said alloy with the diamond crystals in situ to the point where the alloy becomes highly liquid and free-flowing to the point of fluidity, permitting the crystals to adjust themselves in the liquid alloy independently of each other, and then cooling the mixture in the form.

2. A wheel dressing tool comprising a body portion having a socket at one end filled with a mixture of diamond crystals and a matrix alloy, the diamond crystals being sparsely disposed and independently oriented in the direction of the mouth of the socket, said diamond crystals being approximately 30 to the carat and the alloy matrix consisting of silver varying from about 10% to 25%, copper varying from about 67% to about 88%, and phosphorus varying from about 2% to about 8%.

3. A wheel dressing tool comprising a body portion having a socket at one end filled with a mixture of diamond crystals and a fused matrix alloy, the diamond crystals being sparsely and independently oriented in the direction of the mouth of the socket, said diamond crystals being of a size varying from about 25 to 35 to the carat and the alloy matrix consisting of silver, varying from about 10 to 25%, copper varying from about 67 to 88%, and phosphorus varying from about 2 to 8%.

WILLIAM LUDEL.